

# UNITED STATES PATENT OFFICE.

ROBERT A. McDONALD, OF PITTSBURG, PENNSYLVANIA.

## METHOD OF PROTECTING CRUCIBLES.

No. 828,954.

Specification of Letters Patent.

Patented Aug. 21, 1906.

Application filed August 2, 1905. Serial No. 272,322.

*To all whom it may concern:*

Be it known that I, ROBERT A. McDONALD, a resident of Pittsburg, in the county of Allegheny and State of Pennsylvania, have invented a new and useful Improvement in Methods of Protecting Crucibles; and I do hereby declare the following to be a full, clear, and exact description thereof.

My invention relates to the treating of 10 plumbago or carbon crucibles employed in the manufacture of crucible-steel.

One of the great difficulties to be overcome in the manufacture of crucible-steel is to determine with any degree of accuracy 15 just the amount of carbon or silicon which will be found in the finished product, owing to the fact that the molten metal attacks the walls of the crucible and certain proportions of carbon and silicon are given off and find 20 their way into the steel. It is of course impossible to make allowance for these additions of carbon or silicon, as the amounts given off vary with each melting operation. There is no branch of the steel trade that re- 25quires greater accuracy in fixing the quantity of carbon, where in the manufacture of high grades of tool-steel the slightest deviation may make the steel entirely unsuitable for the use to which it is to be applied.

30 The object of my invention is to provide for the treating of the ordinary plumbago or carbon crucibles so as to prevent the throwing of carbon or silicon and making it possible to obtain with great accuracy just the 35 amount of these constituents which will be obtained in the finished product.

To these ends my invention consists, generally stated, in the process of treating ordinary plumbago or carbon crucibles in applying 40 a film of non-carbonaceous material to the inner walls of the crucible after each heat.

To enable others skilled in the art to practice my invention, I will describe the process in detail.

45 In carrying out my process I take the ordinary plumbago or carbon crucible as ordinarily employed, and after the charge of molten metal has been discharged therefrom, and preferably while the crucible is slightly 50 warm, I apply to the interior walls of the crucible a film of clay. In order that the clay will distribute itself properly over the walls of the crucible, I prefer to prepare it in the following manner: The clay is soaked in wa- 55 ter for several days and then run through a sieve to take out any lumps or foreign mat-

ter and in this semiliquid condition when applied to the walls of the crucible will flow over the entire surface, a thin layer or coating adhering to the walls of the crucible, 60 while the surplus settles to the bottom. The application of the clay may be made by introducing into the crucible a sufficient quantity of semiliquid clay. Then by rolling the crucible a sufficient quantity adheres to the 65 walls for the purpose of my invention. It is of course apparent that other means may be employed for applying the coating. The crucible is then allowed to dry, when it is in condition to receive another charge of metal, 70 and when said metal has been melted and discharged from the crucible another coating of clay is applied in the same manner as above.

I may employ any suitable clay for carrying out my invention; but it must be free 75 from carbonaceous material, which if present would unite with the steel, and so affect the accuracy with which the carbon content is determined.

80 While I do not wish to limit myself in any way to the composition of the clay further than that it be free from carbonaceous material, I have found that the following composition gives very successful results: moisture, 85 1.80 per cent.; water of composition, four per cent.; silica, seventy-six per cent.;  $Fe_2O_3$ , 4.45 per cent.;  $Al_2O_3$ , 12.75 per cent.

During the melting process a portion of the film applied as above will appear in the form 90 of a flux or slag on the top of the molten steel and forms a covering or protection against the molten steel taking up oxygen during the period of melting. Practical experience has proven that a thin coating when applied after each heat will act to prevent the throwing 95 of the carbon, sulfur, and silicon. Owing to the fact that the crucible does not throw the carbon, sulfur, and silicon, a better and more regular steel can be produced, for if it is 100 known that the crucible is not throwing carbon then such additions of carbon may be made as necessary, with the result that it is possible to obtain substantially the exact amount of carbon desired in the finished 105 product.

I am aware that it has been proposed to construct crucibles originally with casings or linings of clay; but these have been permanent linings formed at the time that the crucible was made and burned in with the material forming the outer walls of the crucible.

I do not claim such crucibles formed with permanent linings; but my invention is confined to the treating of the crucibles by applying a film of clay or other suitable non-carbonaceous material after each heat.

5 What I claim is—

1. The process of treating ordinary plum-bago or carbon crucibles, consisting in applying to the inner walls thereof after each heat  
10 a film of non-carbonaceous material.

2. The process of treating ordinary plum-bago or carbon crucibles, consisting in applying to the inner walls thereof after each heat a film of clay.

In testimony whereof I, the said ROBERT A. McDONALD, have hereunto set my hand.

ROBERT A. McDONALD.

Witnesses:

ROBERT C. TOTTEN,  
G. C. RAYMOND.